

Aug. 9, 1938.

P. C. SEEL

2,126,350

BACKING PAPER FOR ROLL COATING FILM

Filed April 3, 1937

Fig. 1.



Fig. 2.



Paul C. Seel

INVENTOR

BY *Martin M. Penning*  
*R. Frank Smith*

ATTORNEYS

## UNITED STATES PATENT OFFICE

2,126,350

## BACKING PAPER FOR ROLL COATING FILM

Paul C. Seel, Rochester, N. Y., assignor to Eastman Kodak Company, Rochester, N. Y., a corporation of New Jersey

Application April 3, 1937, Serial No. 134,913

3 Claims. (Cl. 95—9)

This invention relates to photographic roll film backing paper and particularly to a protective coating for such paper.

As is well known, sensitive photographic roll film is ordinarily attached to a sheet of opaque paper and is rolled on a spool together with the paper in order to protect the sensitive surface from the action of light, dust and other agents which would adversely affect it. This opaque 10 backing sheet is customarily coated with a material which renders the sheet impervious to moisture and which does not desensitize or otherwise adversely affect the sensitive layer with which it comes in contact. Various materials have 15 been used for coating the backing paper used in roll film. Cellulose nitrate has been used for this purpose, but it is unsatisfactory because of its high inflammability and its tendency to instability in contact with impurities in the paper. 20 Cellulose organic esters, such as cellulose acetate have also been used. Cellulose acetate, however, is susceptible to moisture and does not give complete protection to the sensitive surface. Fully esterified esters, such as cellulose acetate or cellulose acetate propionate are not as desirable because the choice of solvents from which they may be coated is quite limited, the good solvents being somewhat toxic. Moreover, a serious difficulty is encountered in the use of many of these materials because there is incomplete bonding between the paper and the coating. In many cases the coating is uneven or easily broken and this gives rise to much waste material.

It is, therefore, an object of the present invention to provide an improved backing paper for roll film which is stable in contact with impurities in the paper and which is not highly susceptible to moisture. A further object is to provide a coating which is tightly bonded to the paper and which does not crack or peel when the paper is creased. Other objects will appear from the following description of my invention.

These objects are accomplished by coating the backing paper used in roll film with a layer of a cellulose alkyl ether, such as cellulose ethyl ether having a high alkoxy content.

In the accompanying drawing, Fig. 1 is a sectional view of a portion of a roll film and spool therefor showing the relation of the backing 50 paper to the sensitive film.

Fig. 2 is an enlarged sectional view of the backing paper.

The backing paper is coated according to my invention by applying to it a solution of a cellulose alkyl ether of high alkoxy content from a

suitable solvent. The manner of application of the coating and the manner of drying are non-essential and may be carried out in any suitable way known to the art as long as a thin even coating on the paper is attained.

For example, a 10% solution by weight of cellulose ethyl ether having an alkoxy content of 49.2% is made up in ethylene chloride. This solution is coated on Duplex paper so that a coating approximately .0004" thick is obtained. 10 The coating is then dried at elevated temperature to remove substantially all the solvent from it.

I will now describe my invention by particular reference to the accompanying drawing. In Fig. 1 I have shown a sectional view of a roll film comprising a sensitive film 10 attached to the backing paper 11 by an adhesive strip 12. The backing paper is of sufficient length to protect the sensitive film from light and is attached to the spool 13 at the groove 14.

In Fig. 2 I have shown an enlarged sectional view of a sheet of Duplex paper 15 coated with a layer of cellulose ethyl ether 16. By "Duplex paper" I mean a paper so constructed that two separate sheets, usually differently colored, are bonded together to form a unitary structure. It is to be understood that although this type of paper is usually used, other types may also be employed, according to my invention.

I have referred above to the use of cellulose ethyl ether for coating the backing paper. It is to be understood, however, that other cellulose alkyl ethers may be used, such as cellulose methyl ether. Cellulose alkyl ethers having a wide range of characteristics may be employed. Cellulose alkyl ethers having a high alkoxy content are preferred, since these compounds are only slightly susceptible to moisture. Cellulose alkyl ethers having an alkoxy range of about 42% to 55% may be used, although I am not particularly limited to this range. In order to coat them on the backing paper, the ethers may be dissolved in solvents other than ethylene dichloride, many of which are available, such as acetone, ethyl acetate, butyl acetate, propylene dichloride alone or with methyl alcohol, methyl alcohol alone or with benzene, ethyl alcohol, ethylene glycol mono methyl ether and dioxane.

Various plasticizers and resins may be used if desired such as triphenyl phosphate, diethyl 50 phthalate, mono cresyl para, toluene sulfonate, castor oil, ester gum, gum dammar, etc. These compounds when mixed with the ethers have the effect of increasing the flexibility of the coating.

Among the advantages of cellulose alkyl ethers over backing paper coatings previously used are good adherence to the paper, little tendency to show white lines or cracks when the paper is creased, only slight tendency to pull away from the paper, less sensitivity to abrasion, and a greater tendency to "level out" on the paper when coated, rather than to follow the contours of the paper pattern. All of these advantages produce a superior backing paper coating. Moreover, due to its higher compatibility with other coatings, it may be more conveniently coated over other coatings present on the surface of the paper, such as dye coatings, inks, sizing layers, and the like. Coatings of various thickness may be made by using solutions of various strength and by coating at different speeds. The thickness of the coating is limited only by convenience and economy in application on one hand and by complete protection to the surface of the paper on the other hand. It is to be understood that numer-

ous other modifications may be made within the spirit of my invention, the breadth of which is to be measured by the scope of the appended claims.

What I claim is:

1. A photographic roll film backing paper comprising an opaque paper coated with a layer of cellulose ethyl ether of high ethoxyl content.
2. A photographic roll film backing paper comprising an opaque paper coated with a layer of 10 cellulose ethyl ether having an ethoxyl content of about 49%.
3. A photographic roll film comprising a cel-  
lulosic sheet having on one side thereof a sensi-  
tized layer, and attached to the opposite side 15  
thereof a sheet of opaque paper coated on the  
side opposite that to which the sensitized film is  
attached, with a layer of cellulose ethyl ether  
of high ethoxyl content.

PAUL C. SEEL. 20